

A. F. SULZER,

COMPOSITION FOR MAKING ANTISTATIC PHOTOGRAPHIC FILMS,

APPLICATION FILED MAR. 13, 1922.

1,437,829.

Patented Dec. 5, 1922.

FIG. 1.



FIG. 2.



WITNESS

*Frank H. Stewart.*

INVENTOR

Albert F. Sulzer,  
BY *R. L. Strickfield*

ATTORNEY

Patented Dec. 5, 1922.

1,437,829

# UNITED STATES PATENT OFFICE.

ALBERT F. SULZER, OF ROCHESTER, NEW YORK, ASSIGNOR TO EASTMAN KODAK COMPANY, OF ROCHESTER, NEW YORK, A CORPORATION OF NEW YORK.

## COMPOSITION FOR MAKING ANTISTATIC PHOTOGRAPHIC FILMS.

Original application filed February 21, 1921, Serial No. 446,783. Divided and this application filed March 13, 1922. Serial No. 543,531.

*to all whom it may concern:*

Be it known that I, ALBERT F. SULZER, a citizen of the United States of America, residing at Rochester, in the county of Monroe and State of New York, have invented certain new and useful Improvements in Composition for Making Antistatic Photographic Films, of which the following is a full, clear, and exact specification.

10 This invention relates to a composition of matter useful in the film making art. One object of the invention is to provide a suitable composition which may be incorporated into the film, preferably by forming a layer which will diminish or entirely prevent the formation of static. Other objects will hereinafter appear.

20 Due to the manipulation of sensitive photographic film, some times in manufacture, but more frequently in use, characteristic lines or patches may appear on development, because of electrical discharges which are created during the handling. The fog or fog lines which are thus formed on the film are particularly noticeable in the case of the standard species of motion picture film, which includes a nitrocellulose support or base. It is very important from the commercial standpoint to prevent this defect in 30 the motion picture art, particularly when making negative film strips. The trouble is commonly referred to as "static" and will be so designated herein.

35 While certain camera modifications for preventing this electrical trouble have been proposed, it is very desirable to prevent static by a proper constitution of the film, so that the latter may be employed in any commercial camera without any precautions 40 being taken by the user. Of course, the film should likewise be capable of subsequent fluid treatment and drying on the customary racks or apparatus without injury.

45 I have discovered that film having unexpectedly strong anti-static properties may be prepared by incorporating in its support a layer containing an ether of cellulose and cellulose acetate. This invention is a specific application of the broader discovery disclosed in my co-pending application filed February 21, 1921, Serial No. 446,782.

In the accompanying drawing,—

Fig. 1 is a sectional view on an exagger-

ated scale of the preferred embodiment of my invention;

55 Fig. 2 is a sectional view on an exaggerated scale of a modification of the invention.

In the drawing, 2 represents the support of any customary type, such as a flexible transparent base of nitrocellulose containing softening substances and modifying agents if desired. Upon the support 2 is a photographically sensitive layer 1 which is preferably of the usual silver-haloid emulsion type. 3 is my anti-static layer or backing, this being located, in the preferred form of my invention, on the base or support 2 which is opposite to the sensitive layer 1.

60 The ether-containing layer 3 may be located between the support 2 and sensitive layer 1, as shown in Fig. 2, but this is not the preferred form of my invention, although useful photographic film may be made in that way.

65 In preparing a composition for forming the coating 3, I find it best to dissolve the cellulose ether and the cellulose acetate separately, the two solutions being then mixed and finally diluted if desired. The following proportions and solvents are useful, but, 70 of course, may be widely varied. The proportions are by weight. I may dissolve 45 parts of ethyl cellulose, of the kind which is insoluble in water and not injuriously softened by the latter, in 50 parts of ethyl alcohol and 900 parts of chloroform. I separately dissolve 45 parts of acetone-soluble cellulose acetate in sufficient acetone to make a clear solution. I then combine the acetate and ether solutions into a homogeneous composition. The latter may then be diluted with a mixture of acetone and ethyl alcohol until the acetone content becomes say 4000 75 parts, and the alcohol may amount to 550 parts. By using this method of mixing, a properly diluted flowable composition is provided which sets quickly when coated upon the film support, the volatile ingredients passing away and leaving a transparent, hard anti-static backing resistant to 80 photographic solutions, said coating or backing comprising essentially cellulose ether and cellulose acetate.

85 This application is a division of my prior application, Serial No. 446,783, filed Feb. 21, 1921. 90

100

Having thus described my invention, what I claim as new and desire to secure by Letters Patent is:

1. A composition for forming a layer on an object containing a cellulose ester, said composition comprising a cellulose ether, cellulose acetate, a solvent of said first named ester, and a solvent for cellulose ether, said last named solvent having a stronger solvent action on said ether than said first named solvent.
2. A composition for forming a layer on a photographic film support containing cellulose nitrate, said composition comprising

cellulose ether, cellulose acetate, an amount 15 of a nitrocellulose solvent incapable by itself of fully dissolving said ether, and an amount of a solvent of said ether capable by itself of fully dissolving said ether.

3. A composition for forming a layer on 20 a photographic film support containing cellulose nitrate, said composition comprising ethyl cellulose, cellulose acetate, chloroform, alcohol and acetone.

Signed at Rochester, New York, this 8th 25 day of March, 1922.

ALBERT F. SULZER.